

Jan. 24, 1967

R. W. GATES  
MINIMAL GAS PRODUCING LOW DETONATION RATE EXPLOSIVE  
AND DETONATION SOURCES  
Filed Oct. 2, 1964

3,299,811

*Fig. 1.*



*Fig. 2.*



INVENTOR.  
ROBERT W. GATES

BY  
*Robert A. Anderson*

ATTORNEY

3,299,811

**MINIMAL GAS PRODUCING LOW DETONATION RATE EXPLOSIVE AND DETONATION SOURCES**

Robert W. Gates, Menlo Park, Calif., assignor to the United States of America as represented by the United States Atomic Energy Commission

Filed Oct. 2, 1964, Ser. No. 401,281

16 Claims. (Cl. 102—24)

The present invention relates to explosive compositions and, more particularly, to an explosive composition having a low stable detonation rate and which produces minimal amounts of gaseous reaction products and to sources incorporating such explosive for developing desired energy release profiles.

Explosives, pyrotechnic and propellant compositions have heretofore been provided to supply heat, explosive energy, propulsion forces, shock forces and other desired effects under a wide variety of conditions and to provide a wide variety of explosive effects. However, compositions heretofore provided are unsuitable, for example, as energy sources for simulating events such as the effect of reactivity excursions in order to determine effects thereof on nuclear reactor containment components. Accurate elevation of possible damage from such as excursion using scale models depends largely upon the degree to which excursion conditions including the rate, amount and duration of energy release are validly simulated. A generalized power-time profile of a nuclear power burst or excursion, thought to be characteristic of the energy release causing explosive damage during a runaway excursion is disclosed in the report "Containment Conference at Armour Research Foundation," Chicago, Illinois, May 20-21, 1957 at page 25, and is reproduced hereinafter. The curve is of the exponential form  $P/P_{\max} = e^{at}$  with a time scale such that unit change in time (one period) increases power by a factor of  $e$ . The rising and falling portions of the curve are generally mirror images and are separated by an interval of about two periods during which essentially uniform maximum power is generated. Total effective duration of the burst, wherein about 95% of the total energy is released, approximates seven periods. With typical periods ranging from 1 to 50 milliseconds energy burst durations of from 7 to 350 milliseconds are typical and corresponding total excursion energy estimates range between 200 and 4000  $M_w$ -sec., equivalent to 100 to 2000 lb. of TNT.

Small scale simulation of such an energy release, for example, using a scaling factor of  $1/24$  reduces the foregoing duration limits to 0.3 and 15 milliseconds, respectively. The lower end of such range is appreciably larger than the detonation time of most conventional high explosive events, at least for those involving sizes and amounts of explosive consistent with scaled reactor dimensions and energies. Propellant and pyrotechnic materials, heretofore available, having much slower rates of burning than high explosives, lend themselves to the simulation of long duration excursions; however, they have the serious disadvantage that the rate of energy release is strongly affected by variations of confinement pressure in common with the aforesaid high explosives. There accordingly exists a need for a material with a lower detonation velocity which produces low shock pressures, large amounts of solid and liquid products corresponding to those produced from reactor components by an excursion and appropriate uniform, controllable large total energy releases, and most desirably a wide range of detonation velocities and energy yields.

A composition hereinafter termed "Calpoke" comprising a major proportion of comminuted aluminum metal, a lesser amount of a divalent metal perchlorate and generally smaller amounts of certain high explosive materials

has now been discovered which as a high heat of reaction, will ignite in small diameters as well as large diameter tubes, has a low detonation velocity, and produces only small quantities of gaseous reaction products suitable for simulating nuclear reactor source excursions and runaways under a wide range of duration periods and energy releases as well as other relatively long and sustained duration energy release events. Tube sources containing such composition and adapted to produce desired energy release simulations are also provided.

Accordingly it is an object of the present invention to provide a new and improved explosive of pyrotechnic composition.

Another object of the invention is to provide a low detonation velocity explosive composition which produces minimal amounts of gaseous materials.

Still another object of the invention is to provide an explosive composition having a high heat of reaction, low detonation rate, and produces minimal quantities of gaseous materials suitable for simulating long duration energy release events.

A further object of the invention is to provide a source device employing a low detonation rate explosive to simulate long duration energy release events.

Other objects and advantages of the invention will become apparent from the following description and accompanying drawings, of which:

FIGURE 1, is a power-time profile of typical nuclear reactor excursions, of which curve A is a generalized profile of such a typical excursion, curve B is a stepped source simulation profile and curve C is a simplified rectangular curve profile produced by a simple tube—low detonation rate explosive source in accordance with the invention; and

FIGURE 2 is a source utilizing a low detonation rate explosive composition for producing nuclear reactor excursion energy releases.

The low detonation rate minimal gas producing explosive composition of the invention, i.e., Calpoke, is generally formulated of 10% to 30% by weight of PETN (Pentaerythritol-tetranitrate), 15-35% by weight of calcium perchlorate and 40-60% of comminuted aluminum. Compositions used extensively in simulating nuclear reactor excursions correspond to those in midsections of the aforesaid ranges, i.e., about 20% by weight of PETN, about 25% by weight of calcium perchlorate and about 55% by weight of aluminum which compositions are preferred. Material of the latter composition has a detonation velocity of about 1250 meters/second and releases about 2500 calories/gram of material reacted. The principal reaction products of the explosion are solids or liquids at the detonation temperature, e.g.,  $Al_2O_3$  and metal chloride such as  $CaCl_2$ . Using other admixtures in the ranges set forth above detonation velocities in the range of at least about 1000 to 2000 meters/second and with caloric outputs above and below the above-indicated value can be obtained. Certain other high explosives which can be produced in finely divided forms such as HMX-cyclo 1, 3, 5, 7-tetramethylene 2, 4, 6, 8-tetranitramine RDX-cyclo 1, 2, 5-trimethylene 2, 4, 6-trinitromine, and tetryl-picryl-nitromethylamine can be used in a similar fashion to PETN. Compositions formulated of materials having the foregoing properties are appropriate for the simulation of a wide range of long duration explosive events including the simulation of nuclear reactor runaways with a simple rectangular energy release profile such as curve C of FIGURE 1. Such a profile is produced by a single tube of uniform diameter filled with the composition. Such a source slightly shorter than a model reactor vessel could be used to simulate, e.g., a one millisecond event, providing a simple easily reproducible system for analysis. A stepped source, i.e., variable or stepped diameter sources,

can be used to produce the profile of curve B which more nearly approximates the generalized profile, curve A; however, the use of such a more complicated source configuration possibly cannot be justified since it is not apparent that, for reactor model test purposes, the pressure pulse experienced by the vessel wall is significantly different from that produced by a simple uniform diameter tube source.

For formulating the Calpoke composition PETN or other high explosive mentioned above, in a finely-divided form produced, e.g., by recrystallization is employed. Ignition reliability is improved as the proportions are increased in the range of 10 to 20% (by wt.) and above and detonation velocity is likewise speeded. The calcium perchlorate is generally ground to a very fine consistency under anhydrous conditions and particle sizes of below about 50 microns and preferably below about 35 microns are used. Aluminum in leaf, flake or platelet form is preferred over spherical, needle-like and like forms since it has been found that such materials, often provided as a paint or surface coating pigment, are reliable, safe and inexpensive. Such a material is far superior, for example, to 7 micron diameter spheroidal particles which produced a composition too sensitive to ignition to permit easy compounding and fabrication. Leaf-like, flake, or platelet form aluminum metal having major dimensions of the order of 100 microns have been found satisfactory in practice. However, such materials with major diameter dimensions as small as about 50 microns and larger, e.g., 200 microns and above should generally prove suitable provided that the thickness is not unduly increased. Increasing the proportions of aluminum above stoichiometric proportions tends to reduce the final reaction temperatures and pressures by serving as a heat sink.

A quite wide variety of compositions was investigated in the course of discovering that of the present invention. Initially, compositions containing, by weight, 20% PETN, 48%  $KClO_4$  and 32% and 44% aluminum, respectively (Slowpoke 32), (Slowpoke 44) were found which had a detonation velocity of about 2000 m./sec. and which were believed at first to be suitable to obtain the desired performance. However, damage to test model components was greater than expected or desired. A composition (Slowpoke 56) containing more aluminum, i.e., 56% by weight which therefore contains excess aluminum which tends to lower the reaction temperature produced more favorable pressure and model damage but was too unreliable in smaller grain sizes. Comparative data for various other compositions and that of the invention (Calpoke) are given in Table I which follows.

In view of the differences in fragmentation found to be produced by supposedly identical sources of Pyrocore, Calpoke, and Slowpoke, it became evident that energy output and period were not the only criteria affecting the fragmentation. The actual damage produced is directly caused by the action of pressure upon the vessel wall. Consequently, a series of measurements were made to try to relate the pressure pulse in the vessel to the fragmentation.

10 A steel pressure bomb was constructed with internal dimensions the same as those of the  $\frac{1}{24}$ -scale vessel. Sources of equal energy output and identical periods of the various source materials were detonated in this vessel and attempts were made to measure the pressure produced.

15 Initially, the transducer used to measure the pressure was a Kistler 601, manufactured by the Kistler Instrument Corp. This gage has a high frequency response and a pressure range of from  $\frac{1}{2}$  to 200,000 p.s.i. and low acceleration sensitivity (0.2 p.s.i./g.). The size of the

20 gage was such that it could be fitted into the bomb. The gage appeared to have only one resonance frequency (140 kc.) and it would seem feasible to use it with fair accuracy to a frequency of 30 kc. The transducer element is a quartz crystal which generates an electrical charge proportional to crystal distortion. The measurements are made by determining the voltage this charge generates when placed on a known capacitor. However, for proper response at low frequencies the input impedance must be high. Best results are obtained by using a Kistler ampli-

25 fier-calibrator with the gage.

30 The unfiltered pressure traces first obtained from the helical sources were unreadable even though the readings were taken at the center of the base of the bomb to avoid major oscillations and variations. The only repeatable

35 pressure traces were obtained using a 5 kc. low pass filter. The readings obtained with this filter are not representative of the true wave form, and can only be used to provide a relative measure of the performance of the source materials.

40 This pressure information provides another tool for the examination of source materials with which to extend the working range of the model system. The relatively high detonation velocity of Pyrocore makes it impossible to fabricate the longer period sources. Consequently, it is

45 desirable to have a material with the same energy characteristics as Pyrocore to extend the range so that direct comparisons between the results obtained with the new material and those obtained with Pyrocore are possible. One of the other source materials investigated, i.e., Slowpoke, had all the outward characteristics of Pyrocore but

TABLE I  
*Properties of source materials*

| Source Material       | Detonation Velocity (mm./sec.) | Heat of Reaction (cal./g.) | Smallest Diameter successfully fired (grains/ft.) | Composition                                                              | Relative Pressure Levels |
|-----------------------|--------------------------------|----------------------------|---------------------------------------------------|--------------------------------------------------------------------------|--------------------------|
| MDF                   | 7.3                            | 1,440                      | 0.25                                              | 100% PETN                                                                | 0                        |
| Pyrocore <sup>1</sup> | 4.2                            | 1,560                      | 4                                                 | 20% PETN<br>40% Al<br>40% $BaO_2$<br>20% PETN                            | 1.0                      |
| Slowpoke 32           | 2.0                            | 2,200                      | 12                                                | 32% Al<br>48% $KClO_4$<br>20% PETN<br>44% Al<br>36% $KClO_4$<br>20% PETN | 1.5                      |
| Slowpoke 44           | 1.43                           | 2,436                      | 25                                                | 56% Al<br>24% $KClO_4$<br>20% PETN<br>55% Al<br>25% $Ca(ClO_4)_2$        | 0.75                     |
| Slowpoke 56           | 1.35                           | 2,440                      | 37                                                |                                                                          |                          |
| Calpoke               | 1.25                           | 2,500                      | 8                                                 |                                                                          | 1.0                      |

<sup>1</sup> Values are for 20 grains/ft. Pyrocore. This material is manufactured with different compositions in different core loadings. The composition of the core and consequently its characteristics differ from core loading to core loading.

produced greater damage to models; other materials, Slowpoke-56 and Calpoke, had the same characteristics but produced comparable model change. An investigation of the relative pressures produced by the alternate materials indicated that the high damage producing Slowpoke produced considerably higher pressure during reaction than the other materials. The results of these tests are listed in Table II below.

TABLE II  
*Source material pressure ratios*  
[ALL PRESSURES FROM 5 KC. FILTERED TRACE]

| Shot No. | Material | Peak Pressure (p.s.i.) | Average Peak Pressure (p.s.i.) | Ratio | Simulated         |                |
|----------|----------|------------------------|--------------------------------|-------|-------------------|----------------|
|          |          |                        |                                |       | Energy (Mw.-sec.) | Period (msec.) |
| 111      | SP-56    | 5,800                  |                                |       |                   |                |
| 113      | SP-56    | 11,600                 | 9,666                          | 0.73  | 219               | 0.8            |
| 114      | SP-56    | 11,600                 |                                |       |                   |                |
| 112      | SP-32    | 23,200                 |                                |       |                   |                |
| 116      | SP-32    | 14,500                 | 19,375                         | 1.46  | 219               | 0.8            |
| 120      | SP-32    | 23,600                 |                                |       |                   |                |
| 121      | SP-32    | 16,200                 |                                |       |                   |                |
| 122      | CP-55    | 11,800                 |                                |       |                   |                |
| 123      | CP-55    | 14,700                 | 13,233                         | 1     | 219               | 0.8            |
| 124      | CP-55    | 13,200                 |                                |       |                   |                |
| 126      | PC       | 37,100                 |                                |       |                   |                |
| 127      | PC       | 26,500                 |                                |       |                   |                |
| 128      | PC       | 23,800                 |                                |       |                   |                |
| 129      | PC       | 29,100                 |                                |       |                   |                |
| 146      | PC       | 16,500                 | 26,300                         | 1.99  | 219               | 0.8            |
| 147      | PC       | 27,500                 |                                |       |                   |                |
| 148      | PC       | 22,000                 |                                |       |                   |                |
| 149      | PC       | 28,000                 |                                |       |                   |                |
| 158      | CP-55    | 26,500                 |                                |       |                   |                |
| 159      | CP-55    | 26,500                 | 26,000                         | 1     | 535               | 2              |
| 160      | CP-55    | 25,200                 |                                |       |                   |                |
| 161      | SP-56    | 18,550                 |                                |       |                   |                |
| 162      | SP-56    | 18,550                 | 19,400                         | 0.75  | 535               | 2              |
| 163      | SP-56    | 21,200                 |                                |       |                   |                |
| 164      | SP-32    | 46,400                 |                                |       |                   |                |
| 165      | SP-32    | 34,200                 | 38,300                         | 1.47  | 535               | 2              |
| 166      | SP-32    | 34,200                 |                                |       |                   |                |
| 167      | PC       | 26,500                 |                                |       |                   |                |
| 168      | PC       | 26,500                 | 25,600                         | 0.98  | 535               | 2              |
| 169      | PC       | 23,850                 |                                |       |                   |                |

PC Pyrocore.  
SP Slowpoke.  
CP Calpoke.

The physical dimensions of the sources that would be required to cover the entire range of simulated reactor events are listed in Table III infra. This shows the lengths required to make sources covering the time periods of major interest, and the core loadings required to cover the energy release range for the listed source materials. The table shows that MDF, Pyrocore, and Slowpoke 32 cannot be used for the longer period sources because the lengths involved are much too long to fit into the model vessel. The data also show that Slowpoke 32 and 56 cannot be used for the longer time period sources in the low energy range because the core loading required is less than the core loading of the minimum charge that will sustain detonation. The only material that can be used over the entire range is Calpoke. The versatility of the present composition for use over a wide range of diverse conditions is accordingly demonstrated.

Calcium perchlorate provides several unique advantages in the present composition since, for example, only one mole of  $\text{CaCl}_2$  is produced on detonation as compared to two moles of  $\text{KCl}$ , when a material such as  $\text{KClO}_4$  is used and lower gas pressures are developed on a mole basis even if the  $\text{CaCl}_2$  is vaporized. Moreover,  $\text{CaCl}_2$  has a higher boiling point than does  $\text{KCl}$  so that a higher detonation temperature can be reached without vaporization to

produce gas. Both factors cooperate to reduce the production of gaseous products and the undesirable effects produced by excessive gas pressures on burning rate, etc., which result when perchlorates of monovalent alkali metal, e.g.,  $\text{KClO}_4$  are used instead of a perchlorate of a dibasic or higher valency cation, e.g., a divalent alkaline earth metal is used in the perchlorate, e.g.,  $\text{Ca}(\text{ClO}_4)_2$ . Certain other divalent metal perchlorates can likewise be employed, e.g., those of alkaline earth metals such as Mg and Ba which due to the composite action mentioned above produce solids or only low vapor pressure amounts of chloride reaction products at explosion temperatures. Perchlorates of trivalent metals such as Al and B would produce lesser molar amounts of reaction product chlorides; however, the vaporization temperature of the chlorides of such materials is generally quite low and generally below explosion temperatures so that the bene-

TABLE III  
*Comparison of physical dimensions of sources*

| Source Energy (Mw.-sec.) | Period (msec.) | MDF         |               | Pyrocore    |               | Slowpoke-32 |               | Slowpoke-56 |               | Calpoke     |               |
|--------------------------|----------------|-------------|---------------|-------------|---------------|-------------|---------------|-------------|---------------|-------------|---------------|
|                          |                | Length, in. | Load, gr./ft. | Length, in. | Load, gr./ft. | Length, in. | Load, gr./ft. | Length, in. | Load, gr./ft. | Length, in. | Load, gr./ft. |
| 500                      | 1              | 48          | 22            | 27.5        | 38            | 14.5        | 51.5          | 8.5         | 76            | 8.5         | 74            |
|                          | 2              | 96          | 11            | 55          | 19            | 29          | 25.7          | 17          | 38            | 17          | 37            |
|                          | 8              | 1,384       | 2.8           | 1,220       | 4.7           | 1,116       | 26.4          | 68          | 29.5          | 68          | 9.2           |
| 1,000                    | 1              | 48          | 44            | 27.5        | 76            | 14.5        | 103           | 8.5         | 152           | 8.5         | 148           |
|                          | 2              | 96          | 22            | 55          | 38            | 29          | 51.5          | 17          | 76            | 17          | 74            |
|                          | 8              | 1,384       | 5.5           | 1,220       | 9.5           | 1,116       | 12.8          | 68          | 119           | 68          | 18.5          |
| 3,000                    | 1              | 48          | 132           | 27.5        | 228           | 14.5        | 30.9          | 8.5         | 456           | 8.5         | 444           |
|                          | 2              | 96          | 66            | 55          | 1.4           | 29          | 154.5         | 17          | 228           | 17          | 222           |
|                          | 8              | 1,384       | 16.5          | 1,220       | 28.5          | 1,116       | 38.4          | 68          | 57            | 68          | 55.5          |

<sup>1</sup> Too Long or too big for use.

<sup>2</sup> Less than Failure Diameter.

fits derived from the stoichiometry are offset partially by increased vapor pressures at the reaction temperature. Sources for producing low detonation rate explosions are provided in accordance with the invention as shown in FIGURE 2 of the drawings wherein an elongated ductile metal tube, e.g., lead or 3% antimonial lead, is employed as an exterior case. For some purposes plastic or other tubes can be used as long as the case is impervious to moisture. Normally the tube is of uniform wall thickness and interior diameter but the tube may be tapered, stepped or otherwise shaped to provide desired time-pressure profiles, etc. An insert plug 12, e.g., of methyl methacrylate plastic, is employed to cap one end of tube 11 which plug is provided with a central opening in which is axially disposed electrical detonator 13 (e.g., an M-36 cap) having electrical circuit detonator wires 14. Booster pellets, e.g., of tetryl can be used to improve ignition if some initial accelerated burning rate can be tolerated. Other detonators or detonating lens systems can also be used. The tube 11 is filled with explosive material 16 by a method described below to uniform density and the open end thereof is closed with plastic plug 17. Provision may be made for measuring the longitudinal detonation velocity of the source for monitoring purposes by providing a fine, lightly-insulated resistance wire, e.g., of about 85 ohms/ft. 18 entering the tube 11 at the end distal to said detonator and extending in proximity to the inner wall thereof within explosive 16 to be grounded to the tube 11 at the detonator end. A ground lead 19 affixed to tube 11 may be used to complete the monitoring circuit and measurements may be made as disclosed by A. B. Amster, et al. Review of Scientific Instruments, 31 188-192 (1960). Dimensions and loadings of the preferred composition, supra, for three different scale model sources are set forth in Table IV which follows.

TABLE IV  
*Explosive source data*

| Scale     | "A" Dimension, inches | "B" Dimension, inches | Tube Inner Diameter, inches | Tube Outer Diameter, inches | Grams Per Tube Calpoke |
|-----------|-----------------------|-----------------------|-----------------------------|-----------------------------|------------------------|
| 1/24----- | 8 1/4                 | 8 1/4                 | 0.313±0.015                 | 0.375                       | 9.1                    |
| 1/12----- | 16 1/2                | 17                    | 0.625±0.010                 | 0.749                       | 72.8                   |
| 1/6-----  | 33                    | 34                    | 1.250±0.020                 | 1.500                       | 582.4                  |

The "A" dimension is the distance between emerging ends of resistance wire 18, and dimension "B" is the distance between the inside ends of plugs 12 and 17 of the device shown in Figure 2 of the drawing.

The sensitivity of the composition to ignition and safety during compounding and fabrication is not known with certainty so that remote preparation and loading techniques have been used. Moreover, some of the components are hygroscopic, e.g., calcium perchlorate and low melting so that anhydrous conditions must be used and grinding is somewhat difficult.

The following exemplifies the method compounding and loading the Calpoke composition to provide energy sources described above.

The size reduction was achieved by first drying the calcium perchlorate in vacuum and then putting it through a Mikro Pulverizer in a dry nitrogen atmosphere. This technique produced calcium perchlorate in 35 micron or smaller particles. The aluminum powder was purchased from Cole and De Graf Co. and was designated 333 wa. This material is a common paint pigment and is leaf-like in shape, rather than spherical or needle-like. The largest dimension of the leaves was about 100 $\mu$ . Larger or smaller sizes may be used. This material was used after 7 $\mu$  spherical aluminum particles were found to produce an over-sensitive material. The PETN was recrystallized from acetone-water mixture to form small crystals and passed through a 100 mesh screen.

The three ingredients were weighted in a dry box under

75 dry nitrogen and transferred to a tumbling barrel blender. The blender was heated to 140° F. and a vacuum of 200 $\mu$  pressure was maintained in the blender chamber. These conditions kept the material from absorbing water during mixing. The mixing under vacuum was continued for 45 minutes. The blender was then purged with dry nitrogen and a remote operating valve was attached to the blender. Source tubes 11 were connected to this valve with a length of tygon tubing and purged with dry nitrogen. The valve was opened remotely and the tube filled with Calpoke. The valve was closed and the tube was removed together with its connecting length of tygon, and was capped to exclude air. The tube was then placed in a jolter, and jolted until the Calpoke in the tygon tube had been compacted into the source tube. The tygon tube was then removed and the source tube sealed for use. The tubes were weighed before filling and again after filling to check the amount of Calpoke in each tube. Any tubes which were light or heavy were reprocessed.

20 In model tests a simplified reactor model was used which retained the basic features of actual reactor structures, i.e., pressure vessel, concrete biological shield and access plug. Physical sizes of reactor cores are such that a sealed (1:24) energy source must be contained in a cylindrical volume of 20 cubic inches. A full size reactor vessel 24 feet in diameter and 42 feet high with three inch thick walls may be scaled at 1/24, 1/12 and 1/6 by vessels of 1 ft., 2 ft. and 4 ft. diameter respectively. Sources illustrated in FIG. II and Table IV gave constant velocities of detonation of 1260 m./sec. with no variation as diameter was varied. No scaling effects were noted so that such sources could be used reliably and over a very wide range of conditions. Also, Calpoke detonates at reliable rates without substantial variation from batch to batch, with changes in diameter of changes, change in loading density, and even with varia-

30 35 tions produced with different conditions in tests.

To obtain a visualization of models which might be used, e.g., a 1/24 scale model of the typical reactor above was provided with a 4" I.D. seamless steel tube wall of 0.120" 55 wall thickness with a 1/8" thick 4" diameter bottom and a 1/2" thick steel cap bolted on. A 1/2" high collar was welded about the upper end of the tube for strength. Other scale models in 1/6 and 1/12 scales and a wide variety of experiments beyond the scope of the present disclosure 60 were performed using such models.

While there has been described in the foregoing what may be considered to be preferred embodiments of the invention modifications may be made therein without departing from the teachings and scope of the invention 65 and it is intended to cover all such as fall within the scope of the appended claims.

What is claimed is:

1. A minimal gas producing low detonation rate explosive composition comprising a minor proportion of a high explosive in intimate admixture with a greater proportion of a perchlorate of a metal having a valency of at least two and which produces a chloride having a low vapor pressure at the explosion temperature, and a major proportion of particulate aluminum metal.
2. A low detonation rate minimal gas producing explo-

sive composition comprising high explosive in an amount in the range of about 10 to 30% by weight, about 15 to 35% by weight of a perchlorate of a metal being divalent at least and which produces a chloride reaction product having a low vapor pressure at the explosion temperature, and about 40 to 60% by weight of aluminum, said high explosive, perchlorate and aluminum being in a uniform finely-divided intimate composite admixture.

3. An explosive composition as defined in claim 2 wherein said high explosive is a material selected from the group consisting of PETN, HMX, RDX and tetryl.

4. An explosive composition as defined in claim 2 wherein said perchlorate is a metal selected from the group consisting of calcium, magnesium and barium.

5. An explosive composition as defined in claim 2 wherein said aluminum is in the form of leaf-like particles.

6. A low detonation rate minimal gas producing explosive composition comprising a high explosive selected from the group consisting of PETN, HMX, RDX and tetryl in an amount in the range of about 10 to 30% by weight, a perchlorate of an alkaline earth metal selected from the group consisting of calcium, magnesium and barium in an amount in the range of about 15 to 35% by weight, and leaf-like aluminum powder in an amount in the range of about 40 to 60% by weight, said high explosive being in a uniform finely-divided intimate composite admixture.

7. A composition as defined in claim 6 wherein said aluminum powder has a major diameter dimension of the of 100 microns.

8. A low detonation rate minimal gas producing explosive composition comprising a high explosive selected from the group consisting of PETN, HMX, RDX and tetryl in an amount in the range of about 10 to 30% by weight, calcium perchlorate in an amount in the range of about 15 to 35% by weight, and leaf-like aluminum powder in the range of about 40 to 60% by weight, said high explosive, perchlorate and aluminum powder being in a uniform finely-divided intimate composite admixture.

9. A composition as defined in claim 8 wherein said high explosive is PETN.

10. A low detonation rate minimal gas producing explosive comprising about 10 to 30% by weight of PETN, about 15-35% by weight of calcium perchlorate and 40-60% by weight of finely-divided leaf-like aluminum metal particles, said PETN, calcium perchlorate and aluminum metal particles being in a uniform intimate composite admixture.

11. A low detonation rate minimal gas producing explosive comprising about 10 to 30% by weight of PETN, about 10-35% by weight of calcium perchlorate and 40-60% by weight of finely-divided leaf-like aluminum metal particles, said PETN, calcium perchlorate and aluminum metal particles being in a uniform intimate composite admixture.

12. A source for producing relatively long duration explosive events with minimal gas production comprising an elongated tubular closed casing member, a compacted intimate admixed composite explosive including a high explosive in an amount in the range of about 10 to 30% by weight, about 15 to 35% by weight of a perchlorate of a metal ion of at least divalency and productive of a chloride reaction product of said metal having a low vapor pressure, and about 40 to 60% by weight of finely-divided leaf-like particles of aluminum metal disposed in said casing, and detonator means disposed in contact with said explosive in said casing.

13. A source for producing relatively long duration explosive events with minimal gas production comprising an elongated tubular closed casing member, a compacted intimate admixed composite explosive including a high explosive selected from the group consisting of PETN, HMX, RDX and tetryl in an amount in the range of about 10 to 30% by weight, about 15 to 35% by weight of a perchlorate of a metal ion of at least divalency and productive of a chloride reaction product of said metal having a low vapor pressure, about 40 to 60% by weight of finely-divided leaf-like particles of aluminum metal disposed in said casing, and detonator means disposed in contact with said explosive in said casing.

14. A source for producing relatively long duration explosive events with minimal gas production comprising an elongated tubular closed casing member, a compacted intimate admixed composite explosive including a high explosive in an amount in the range of about 10 to 30% by weight, about 15 to 35% by weight of a perchlorate of a metal selected from the group consisting of calcium, magnesium and barium and productive of a chloride reaction product of said metal having a low vapor pressure, and about 40 to 60% by weight of finely-divided leaf-like particles of aluminum metal disposed in said casing and detonator means disposed in contact with said explosive in said casing.

15. A source for producing relatively long duration explosive events with minimal gas production comprising an elongated tubular casing member, a compacted intimate composite admixture of PETN in an amount in the range of about 10 to 30% by weight, about 15 to 30% by weight of calcium perchlorate, and about 40 to 50% by weight of aluminum powder of leaf-like particulate form, disposed in said casing, means for closing said casing, and detonator means disposed in contact with said explosive.

16. A source as defined in claim 15 wherein said PETN is present in the amount of about 20% by weight, said calcium perchlorate in an amount of about 25% by weight and said aluminum particles in an amount of about 55% by weight.

No references cited.

55 BENJAMIN R. PADGETT, Primary Examiner.